

## UNITED STATES PATENT OFFICE

2,354,662

## METHOD OF SIZING PAPER

Robert S. Bryce, Rochester, N. Y., assignor to  
Eastman Kodak Company, Rochester, N. Y., a  
corporation of New Jersey

No Drawing. Application July 16, 1941;  
Serial No. 402,719

6 Claims. (Cl. 117—156)

This invention relates to a method of sizing paper with gelatin and a dihydroxymethyl urea.

In the manufacture of paper it is oftentimes desirable to pass the paper through a solution of animal glue or gelatin to increase certain of the physical characteristics of the paper, such as water resistance, wet strength and smoothness. Often, at the present time, this gelatin is hardened by passing the paper sheet, after treatment with the gelatin, through a solution of formaldehyde and/or chromium salts, or by fuming the paper with formaldehyde. Fuming of the paper, sized with gelatin, with formaldehyde results in decidedly higher wet strength and greater blister resistance than hardening of gelatin size by passing it through a water solution of formaldehyde. This fuming operation, however, necessitates an extra step in the manufacturing process and the use of additional equipment.

An object of this invention is to provide a method of sizing paper, having a wet strength and blister resistance, comparable to that of gelatin-sized paper which has been treated with formaldehyde gas but without the necessity of an extra step in the process and additional equipment in carrying it out. Another object of this invention is to provide a method of fuming the gelatin size of a paper sheet with formaldehyde from within the sheet during the processing operation. Other objects of my invention will appear herein.

I have found that by incorporating one of the class of dihydroxymethyl ureas, such as dihydroxymethyl urea, dihydroxymethyl thiourea and dihydroxymethyl guanidine in a gelatin sizing solution for paper that the gelatin size is hardened within the paper upon the application of heat, such as in the drying operation making the paper. I have found that the resulting paper has a much higher wet strength and greater blister resistance than obtained when a paper sheet containing gelatin size is subjected to the action of an aqueous formaldehyde solution and that this invention permits the fuming of the paper sheet with formaldehyde fumes without a fuming box. Obviously the gelatin and the dihydroxymethyl urea may be applied to the paper from separate solutions prior to the heat treatment.

The dihydroxymethyl ureas exert a hardening effect upon gelatin sizing if used in any amount up to the limit of solubility in the sizing composition. As, however, there is a tendency for this type of compound to form resins, it is preferred that only sufficient dihydroxymethyl urea be used

to give the desired results (ordinarily within the range of 0.5—5% and preferably not more than 3%), as too great an amount of resin in the paper will make for brittleness. In cases where brittleness is not objectionable or is even desirable, larger proportions of a dihydroxymethyl urea may be employed.

Formaldehyde is liberated from a dihydroxymethyl urea by the action of heat. Heat is ordinarily applied to a paper sheet when it is passed over hot drying drums and use may be made of this heat in liberating formaldehyde from the dihydroxymethyl urea in the sizing composition of this invention. The gelatin is hardened in this operation by the liberated formaldehyde. As a heat operation is necessary to liberate formaldehyde in accordance with my invention, any temperature, which will liberate formaldehyde from a dihydroxymethyl urea without decomposing the cellulose of the paper sheet, may be employed. The literature states that dihydroxymethyl urea loses water and formaldehyde when subjected to a temperature above its condensation point. The temperatures ordinarily employed for the hot drying drums in paper manufacture such as 220—240° F. may be employed with entire satisfaction in this process.

If the ordinary drying of the paper does not give a paper of the desired wet strength, the time of treatment may be lengthened such as by passing the paper over the rolls more slowly or a catalyst may be incorporated in the sizing composition to speed up the liberation of formaldehyde and hardening of the gelatin. As a rule incomplete hardening of the gelatin size is sufficient in most instances to give a paper of satisfactory wet strength. Upon storage the wet strength of paper in which the size is incompletely hardened continues to increase due probably to further hardening of the gelatin occurring.

In hardening gelatin, in accordance with this invention, the use of the technical grade of dihydroxymethyl urea is ordinarily satisfactory. For instance, in the case of dimethylol urea, the commercial grade may be employed even though there may also be present therein monomethylol urea and some polymeric material as well as small amounts of formaldehyde and urea. Dimethylol urea slowly transforms itself from the monomeric to the polymeric form upon standing at normal temperatures so that even if the material initially on hand is 100% monomer, a measurable quantity of polymer will be present if the dimethylol urea has been standing for a short time before use. This condensation proceeds upon standing

at such a rate that after a few months the dimethylol urea is no longer water soluble and hence cannot be used. The presence of polymeric dimethylol urea does not interfere with the hardening action of the monomeric compound providing there is not enough of the polymer present to render the dimethylol urea, incapable of being dispersed in water.

The dihydroxymethyl ureas generally are suitable for use in hardening gelatin, as described herein. If the paper is to be used for some specific purpose, it may be that one particular dihydroxymethyl urea will be found to be more suitable than others. For instance, for paper upon which a photographic emulsion is to be coated, I have found that dimethylol urea is particularly suitable due to its complete inertness thereto. If desired, a mixture of these hardening agents may be employed in the sizing solution or other materials, such as hexamethylene tetramine, may also be incorporated in the sizing solution along with the dihydroxymethyl urea if desired.

Although the proportion of gelatin in sizing compositions in accordance with my invention may be varied as desired, as a practical matter the usual proportions of gelatin used will be within the range of 2% to 10% because when more than 10% of gelatin is used the sizing composition is ordinarily too viscous unless a low viscosity gelatin is employed and a proportion of gelatin less than 2% does not have a sufficiently pronounced sizing effect for most purposes.

A sizing composition of gelatin and water containing a dihydroxymethyl urea is suitable for sizing both papers made from wood fiber and those made from rag fiber as well as papers made using a mixture of those fibers. For instance, in a machine scale operation in which 100% wood fiber was used, the paper was tub sized with an aqueous solution containing 4½% gelatin and 3% dimethylol urea, in addition to formaldehyde and chromium salts. After drying the paper by passing over hot drying drums, the wet strength was found to be 17 as compared to 9 for paper sized in the same manner except that the dimethylol urea was omitted. In another instance, a machine scale experiment was carried out in which 100% rag fiber was used and the paper was sized with a water solution containing 4½% gelatin and 1% dimethylol urea in addition to formaldehyde and chromium salts. The paper, which was dried by passing over the hot drying drums, showed a wet strength of 40 as compared to 16% for similar paper sized in the same manner with gelatin hardened with formaldehyde but in which the dimethylol urea was omitted. In a third case using 100% rag fiber and but 3% dimethylol urea, the other conditions being the same as before, a paper, having a wet strength of 47, was obtained, as compared to 16% for the paper sized for formaldehyde hardened gelatin. An improvement in blister resistance was noted in all cases.

The following example illustrates the sizing of paper in accordance with this invention. A sizing bath composed of 4.25 parts of gelatin, 1.1 parts of dimethylol urea, 94.65 parts of water was prepared as follows: The gelatin was soaked in a small proportion of cold water until it was completely swollen. Hot water was then added to dissolve the gelatin. The dimethylol urea was then added in the form of a 20% water solution and the remainder of the water was then added.

Paper was sized by passing a long sheet of it continuously through a tub containing the sizing composition specified pressed between press

rolls to remove excess size and immediately passed over hot drying drums where the paper is dried and formaldehyde is liberated from the dimethylol urea. A paper having a good blister resistance and wet strength was obtained.

Sometimes to speed up or catalyze the decomposition of the dihydroxymethyl urea, it is desirable to add a small amount of an acid or acidic salt as the catalyst, to the solution. Although quantities of acid or acidic salt greater than 1%, such as up to 3% may be effective, it is preferred to use a quantity of decomposition catalyst less than 1% in the excess bath. The water-soluble salts of weak bases and strong acids are particularly good for this purpose. For instance, an amount of aluminum sulfate of approximately 0.08% works quite satisfactory in this connection. If in the above-given sizing composition a small proportion of aluminum sulfate is incorporated, the decomposition of the dimethylol urea therein is accelerated when the paper containing it is passed over drying drums. Some catalysts which may be employed instead of aluminum sulfate are ammonium chloride, zinc chloride, sulfuric acid, hydrochloric acid, sodium bisulfate, phosphoric acid and acetic acid. The reaction in this invention proceeds at a good rate under mildly acid conditions and any compound which will lower the pH of the sizing composition and which is compatible with the conditions of operation will serve as a catalyst in this invention.

I have found that the wet-strength imparting properties of a mixture of gelatin and a dihydroxymethyl urea accompanied by heat treatment is much greater than would be expected from the wet-strength imparting properties of each separately. For instance a paper which without any sizing gives a wet strength of 6 was sized with gelatin alone (4½% solution in water). A product having a wet strength of 10½ was obtained. When the paper instead of being sized with gelatin, was sized with dimethylol urea (1% solution in water) followed by heat treatment to polymerize the monomer, a paper having a wet strength of 10½ was obtained. A sample of this paper which has a wet strength of 6, unsized, was sized with an aqueous solution of a mixture of gelatin and dimethylol urea instead of one or the other alone. The sizing solution contained 4½% of gelatin and 1% of dimethylol urea together with a small amount of aluminum sulfate as the catalyst. The paper was subjected to a drying operation by passing over warm rolls. It was found to have a wet strength of approximately 50. As pointed out above the same result would be obtained without the catalyst with a longer drying or heat treatment.

Paper prepared in accordance with my invention due to its high wet strength and blister resistance is adapted particularly to uses involving immersion such as for photographic or photostatic purposes in which the products are treated in developing, fixing and/or washing baths. Any other product which is subjected to water or dampness may with advantage be prepared from paper sized in accordance with this invention.

I claim:

1. A method of sizing paper which comprises treating it with gelatin and a dihydroxymethyl urea both in dilute aqueous solution and subsequently subjecting the paper to a temperature which will liberate formaldehyde from the dihydroxymethyl urea without decomposing the cellulose of the paper.

2. A method of sizing paper which comprises treating it with water containing 2%-10% of gelatin and 0.5-5% of a dihydroxymethyl urea both in solution therein and subsequently subjecting the wet paper to a temperature which will liberate formaldehyde from the dihydroxymethyl urea without decomposing the paper.

3. A method of sizing paper which comprises treating it with water containing 2%-10% of gelatin and 0.5-5% of a dihydroxymethyl urea together with a small amount of an acidic catalyst all in solution therein and subsequently subjecting the wet paper to a temperature which will liberate formaldehyde from the dihydroxymethyl urea without decomposing the paper.

4. A method of sizing paper which comprises treating it with water containing 2%-10% of gelatin, 0.5-5% of a dihydroxymethyl urea and a small amount of aluminum sulfate all in solu-

tion therein and subsequently subjecting the wet paper to a temperature which will liberate formaldehyde from the dihydroxymethyl urea without decomposing the paper.

5. A method of sizing paper which comprises treating it with water containing 2%-10% of gelatin and 0.5-5% of dimethylol urea both in solution therein and subsequently subjecting the wet paper to a temperature which will liberate formaldehyde from the dimethylol urea without decomposing the paper.

10 6. A method of sizing paper which comprises treating it with water containing approximately 4½% gelatin and 1-3% of dimethylol urea both in solution therein and subsequently subjecting the wet paper to a temperature which will liberate formaldehyde from the dimethylol urea without decomposing the paper.

ROBERT S. BRYCE.